

# United States Patent

[19]

d'Albignac et al.

[11] 3,811,836

[45] May 21, 1974

[54] **CONTINUOUS DYEING OF SYNTHETIC TEXTILE FIBRES WITH A BASIC CHARACTER**

|           |        |                    |       |
|-----------|--------|--------------------|-------|
| 3,170,757 | 2/1965 | Gift et al.....    | 8/173 |
| 3,265,461 | 8/1966 | Luitzel et al..... | 8/173 |

[75] Inventors: **Jean Marie Louis Jules d'Albignac; Jean-Francois Gamaury, both of Creil, France**

*Primary Examiner*—Leon D. Rosdol

*Assistant Examiner*—T. J. Herbert, Jr.

*Attorney, Agent, or Firm*—Browne, Beveridge, De-Grandi & Kline

[73] Assignee: **Societe Civile Soltex, Paris, France**

[22] Filed: **Dec. 20, 1971**

[21] Appl. No.: **210,269**

## Related U.S. Application Data

[63] Continuation of Ser. No. 847,000, July 29, 1969, abandoned.

## Foreign Application Priority Data

Aug. 14, 1968 France ..... 68,162965

[52] U.S. Cl. .... **8/173, 8/93, 8/176**

[51] Int. Cl. .... **D06p 5/04**

[58] Field of Search..... **8/173, 93, 176**

## References Cited

### UNITED STATES PATENTS

3,169,822 6/1965 Randall..... 8/54 X

[57]

## ABSTRACT

Dyebath comprising a solution of anionic dyestuff possessing at least one free acid group in an organic liquid, the boiling point of the organic liquid being from 120°C. to 300°C. and a process for the continuous dyeing of synthetic textile fibres possessing basic functions in which the fibres are passed for from some seconds to some minutes at a temperature from 90°C. to 160°C. through a solution comprising an organic liquid having a boiling point from 120°C. to 300°C. and an anionic dyestuff in the form of the free acid.

**2 Claims, No Drawings**

## CONTINUOUS DYEING OF SYNTHETIC TEXTILE FIBRES WITH A BASIC CHARACTER

This is a continuation, of application Ser. No. 847,000, filed July 29, 1969, now abandoned.

The present invention concerns the continuous dyeing of synthetic textile fibres with a basic character.

Textile fibres consisting of synthetic polyamides are usually dyed either in aqueous solutions or dispersions of dyestuffs at the boiling temperature of the water or under pressure at temperatures between 100°C. and 130°C. or by foularding in an aqueous suspension of dyestuff followed by thermal fixation or steaming.

These processes have various disadvantages. In the case of the polyamides 11 they lead, for example, to dyeings which are not very deep, and in the case of textured polyamides, they lead to uneven shades. Further, when water-insoluble plasto-soluble dyestuffs are used, expensive grinding and dispersing operations are required in order to obtain these dyestuffs in a suitable form.

In order to remove these disadvantages, it has been proposed to dye these fibres by impregnating with a solution of dyestuff in a mixture of alcohols and halogenated hydrocarbon derivatives followed by a heat treatment. There are however great technical difficulties in the application of this process, especially in obtaining shades which are uniform and fast to rubbing.

It has also been proposed to dye with solutions of dyestuffs in non-volatile solvents and at elevated temperature; however, this technique, if used with the usual commercial dyestuffs, does not give satisfactory results, especially with regard to the tinctorial yields and the fastness to wet treatments and to rubbing.

We have now found that excellent results are obtained in the continuous dyeing of synthetic textile fibres having basic functions by passing these materials for a very short time from some seconds to some minutes, preferably between 10 seconds and 2 minutes, at a temperature from 90°C. to 160°C. through a solution comprising an organic liquid with a boiling point from 120°C. to 300°C. and an anionic dyestuff in the form of the free acid.

The synthetic textile fibres possessing basic functions to which the present process is applied may be for example, based on polyamides (condensation products of hexamethylenediamine with adipic acid, polymerisation products of  $\epsilon$ -caprolactam, polycondensation products of amino-undecanoic acid and other analogous products), or based on polyurethanes. They may be in various forms such as fabrics, jersey, or yarns, and they may or may not be textured.

The dyestuffs which may be used are those containing at least one free acid group not in salt form, such as for example a sulphonate or carboxylic acid group. Nonmetallised dyestuffs or metalliferous complexes of the 1/1 type or the 1/2 type possessing free acid groups may for example be used. The amounts of dyestuff to be used depend upon the dyeing conditions and the shades required; they are only limited by the solubility of the dyestuffs in the bath.

Suitable organic liquids which boil at between 120°C. and 300°C. and which may be used as solvents for the dyestuffs are, for example, diols and triols such as ethylene glycol, propylene glycol, diethylene glycol and glycerine.

The application of the solution of dyestuff to the textile material is preferably effected by impregnation and circulation, for example, in an apparatus of the wheeled vat type or in a William unit. The greater part of the excess solution may be eliminated by squeezing, for example by squeezing between two rollers and is preferably returned to the impregnating bath.

The textile material is then washed, either in the cold or hot, with a solvent or a mixture of solvents with a low boiling point, such as methanol, ethanol, isopropyl alcohol, acetone, methyl ethyl ketone, methylene chloride, or methyl or ethyl acetate. These volatile solvents may be easily recovered and recycled.

The present process enables colorations to be obtained in very short times which have penetrated well and are bright, resistant to rubbing and have a fastness to wet treatments and light at least equal to those obtained by the usual processes. It also enables the dyestuffs to be used in any physical form and the long grinding necessary to obtain some of them in a form suitable for their usual application to be avoided.

The invention is illustrated by, but not limited to, the following Examples in which the parts are parts by weight.

25

### EXAMPLE 1

10 parts of the dyestuff C.I. Acid Blue 129 (Color Index No. 62058), in the form of the acid, are dissolved at about 100°C. in 1000 parts of pure ethylene glycol. 30 This solution is raised to a temperature of 110°C. and a polyamide-6 fabric is moved about therein for one minute, then drained by squeezing between two rollers, and immediately rinsed in acetone. A deep and uniform blue shade is thus obtained having a fastness to rubbing, washing and light comparable to that obtained by dyeing in an aqueous bath.

If, instead of the dyestuff mentioned above, one of those indicated in Table I below is used in the form of the free acid, the dyeing conditions remaining the same, uniform and well developed shades are also obtained.

TABLE I

|                                                                                                                                                      | Dyestuff       | Shade |
|------------------------------------------------------------------------------------------------------------------------------------------------------|----------------|-------|
| C.I. Acid Green 25 (Color Index No. 61750)                                                                                                           | green          |       |
| C.I. Acid Red 57 (reaction product in acid medium of diazo derivative of (N,N-diethylsulphamoyl)-2 aniline with amino-2 naphthol-8-sulphonic-6 acid) | red            |       |
| C.I. Acid Yellow 25 (Color Index No. 18835)<br>N,N'-bis (1-amino-2-sulpho-4-anthraquinonyl)-4,4'-diamino-3,3',5,5'-tetra-methyl-diphenyl-methane     | yellow<br>blue |       |

### EXAMPLE 2

55 10 parts of the dyestuff C.I. Acid Blue 129 in the form of the acid are dissolved at about 100°C in 1,000 parts of diethylene glycol. This solution is raised to a temperature of 120°C. and a polyamide-6 fabric is moved about therein for one minute, then drained by squeezing between two rollers and rinsed immediately in acetone. A result comparable to that obtained in the first paragraph of Example 1 is obtained.

### EXAMPLE 3

65 20 parts of the dyestuff C.I. Acid Blue 129 in the form of the acid are dissolved in about 100°C. in 1,000 parts of glycerine. This solution is raised to a tempera-

ture of 110°C. and a polyamide-6 fabric is dyed therein as in Example 1, a similar result being obtained.

## EXAMPLE 4

On replacing the polyamide-6 fabric in Example 1 by a polyamide 6-6 fabric and operating at 130°C. instead of 110°C. a uniform blue shade having good fastness to washing and rubbing is also obtained.

We claim:

1. Dyebath consisting of a polyol having a boiling point from 120°C. to 300°C. in which is dissolved an acid dyestuff containing a sulphonic or carboxylic acid group in the form of the free acid.

5

10

10

2. Process for the continuous dyeing of synthetic textile fibres possessing basic functions in which the fibres are passed for from 10 seconds to 2 minutes at a temperature from 90°C. to 160°C. through a solution consisting of a polyol having a boiling point from 120°C. to 300°C. and a polyol soluble acid dyestuff containing a sulphonic or carboxylic acid group in the form of the free acid, then squeezed out, and finally rinsed with a solvent selected from the group consisting of methanol, ethanol, isopropyl alcohol, acetone, methyl ethyl ketone, methylene chloride, methyl acetate and ethyl acetate.

\* \* \* \* \*

15

20

25

30

35

40

45

50

55

60

65